

[54] METAL HALIDE DISCHARGE LAMP  
HAVING HEAT ABSORBING COATING[75] Inventors: William I. Bamberg, Medford;  
William M. Keeffe, Rockport, both  
of Mass.[73] Assignee: GTE Sylvania Incorporated,  
Danvers, Mass.

[22] Filed: June 3, 1974

[21] Appl. No.: 475,733

[52] U.S. Cl. .... 313/44; 117/215; 117/221;  
117/124 A; 313/47; 313/221; 313/220; 313/45[51] Int. Cl.<sup>2</sup> .... H01J 61/52[58] Field of Search .... 313/45, 44, 47, 221, 220;  
117/215, 221, 124 A

[56]

## References Cited

## UNITED STATES PATENTS

3,842,304 10/1974 Beyer et al. .... 313/44

Primary Examiner—R. V. Rolinec

Assistant Examiner—Darwin R. Hostetter

Attorney, Agent, or Firm—James Theodosopoulos

[57]

## ABSTRACT

The arc tube ends of a metal halide lamp have a double layer coating thereon, the first coating being a heat absorbing coating and the second coating being a heat reflective coating.

6 Claims, 1 Drawing Figure





## METAL HALIDE DISCHARGE LAMP HAVING HEAT ABSORBING COATING

### THE INVENTION

This invention relates to high intensity metal halide arc discharge lamps. Such lamps comprise an arc tube, usually made of fused quartz or other high silica glass, having electrodes disposed at its ends and containing a fill including an inert starting gas, mercury and one or more metal halides. The mercury is completely vaporized during normal lamp operation while the metal halides are usually only partially vaporized.

The arc tube press sealed ends of such lamps usually have a heat reflective coating thereon in order to maintain said ends at a sufficiently high temperature so as to ensure adequate vapor pressure of the metal halides in the arc tube. Examples of such coatings are shown in U.S. Pats. Nos. 3,325,662 and 3,374,377, which disclose coatings of calcium pyrophosphate and zirconium dioxide.

However, in spite of these heat reflective coatings, usually white, the area behind the electrodes is usually the coolest part of the arc tube. This results in condensation of the low vapor pressure metal halides thereat, after lamp extinguishment. Since a crevice usually exists in the quartz glass at the junction of the electrode assembly with the press seal, the metal halides often condense out within the crevice. Once this occurs, there is little chance for the crevice area to reach a high enough temperature to drive these condensed halides back into the arc tube where they would be available to the arc discharge.

High intensity metal halide discharge lamps are generally formulated to include quantities of several different metal halides which, given the operating conditions within the arc tube and vapor pressure characteristics of the halides, will insure the correct partial pressures of the halides in the discharge to cause the arc to radiate with the desired spectral characteristics. If a portion of the metal halide fill is lost into the crevice region, the spectral characteristics of the discharge change. Not only is the total quantity of available metal halide reduced by condensation, but also the chemical balance of the remaining halide fill is changed from optimum, since the different vapor pressure characteristics of each fill component cause crevice condensation out of proportion to the desired balance in the arc discharge tube.

A purpose of this invention is to eliminate such crevice condensation and thereby obviate changes in the discharge spectral characteristics resulting therefrom during lamp life.

This is accomplished by first coating the region behind the electrodes, or at least in the immediate area of the crevice formation, with a dark or gray coating. Such a coating is a better heat absorber than the heat reflective coatings of the prior art. Then, in order to prevent heat loss by reradiation from the first coating, a second heat reflective coating is directly deposited onto the first coating. This second coating can be a white prior art coating.

An embodiment of this invention is shown in FIG. 1 which is an elevational view of a metal halide arc discharge tube. Arc tube 1 has press seals 2 at each end thereof. At each end of arc tube 1 are electrodes 3 which are supported by lead-in wires 4. Lead-in wires

4 extend into and are embedded in press seals 2. The previously mentioned crevice exists at the point where lead-in wire 4 enters press seal 2. Lead-in wires 4 are connected to a molybdenum ribbon 5, embedded 5 within press seal 2, to which external lead-in wires 6 are connected. A starting electrode 7, connected to an external lead-in wire 8, is also located at one end of arc tube 1.

Coating 9, which covers the ends of arc tube 1 behind electrodes 3, extends from about the vicinity of electrodes 3 onto press seal 2. Coating 9 comprises a first coating of a dark or gray material, on top of which a second coating of white heat reflective material is deposited. In one example, this first coating consisted of 10 a mixture of zirconium diboride ( $ZrB_2$ ) and zirconium dioxide ( $ZrO_2$ ) while the second coating consisted of 15  $ZrO_2$ .

Several 400 watt metal halide lamps having an arc tube coating in accordance with this invention were 20 evaluated and compared with control lamps having only the prior art white reflective coating. All arc tubes contained a fill of 51 mg mercury, 5.0 mg mercuric iodide, 20 mg sodium iodide, 0.7 mg scandium, 0.5 mg thorium and 27 torr argon. This fill is designed to yield 25 high lamp efficacy with good white light, that is, light having a high color rendering index.

The lamps in accordance with this invention yielded 35,600 lumens initially versus 33,200 for the control lamps. After 6000 hours operation, the lamps of this 30 invention yielded 24,500 lumens, for a lumen maintenance of 70%. The control lamps had dropped to 21,300 lumens, a lumen maintenance of only 61%.

An analysis of the radiation intensity of the various 35 fill components of the 6000 hour operated lamps was made in order to compare the changes between the two sets of lamps. The analysis was made by comparing the ratio of the intensity of the spectral lines which are characteristic of the particular metals in the fill to the 40 intensity of the 4358 angstrom mercury line. The ratio of the 5896 sodium line to the 4358 mercury line was 0.213 for the lamps of this invention versus 0.133 for the control lamps. For the 5688 and 5682 sodium lines, said ratios were 0.174 and 0.094, respectively, for 45 lamps of this invention, as against 0.055 and 0.028 for the control lamps. The 4499 thorium line had a ratio of 0.211 for the invention lamps and 0.138 for the control lamps. For the 4734 scandium line, the ratios were 0.356 and 0.188, respectively. These results show that 50 there was proportionately more sodium-thorium-scandium radiation from the invention lamps, after 6000 hours operation, than there was from the control lamps; thus there was less condensation of the iodides of sodium, thorium and scandium in the invention lamps than there was in the control lamps.

The only spectral line, of those analyzed, which 55 showed a higher ratio in the control lamps than in the invention lamps was the 5770 mercury line. The ratio of the 5770 mercury line to the 4358 mercury line was 0.043 in the invention lamps and 0.062 in the control 60 lamps. The reason for this is that as the various metal halides condense out in the arc tube, the radiation characteristics of the arc discharge more closely approach those of a mercury discharge, with its relatively low efficacy, blue-green radiation and higher arc temperature.

In order to determine if the arc temperature of the 65 control lamps, after 6000 hours, was higher than the

arc temperature of the invention lamps, the ratios of ionized to atomic radiation for scandium and thorium were determined. Higher concentration of ions indicates a higher arc temperature. The ratio for thorium was determined by comparing the intensity of the 4391 thorium ion line with the 4499 thorium atom line; for scandium, the 4374 scandium ion line was compared with the 4734 scandium atom line.

Said ratio for thorium was 0.632 for the invention lamps and 1.071 for the control lamps. For scandium the ratios were 0.724 and 1.089, respectively. This confirms the higher arc temperature characteristic of a mercury discharge lamp, and the increased condensation of the metal halide additives, in the prior art control lamps.

In these lamps, the dark coating consisted of 25%  $ZrB_2$  and 75%  $ZrO_2$ . The coating was applied from a suspension prepared by mixing the necessary quantities of a  $ZrB_2$  suspension and a  $ZrO_2$  suspension to yield a suspension containing 25%  $ZrB_2$  and 75%  $ZrO_2$ . The  $ZrB_2$  suspension consisted of 50 grams  $ZrB_2$ , 1.25 grams colloidal alumina and 1000 ml isopropyl alcohol. The  $ZrO_2$  suspension consisted of 2000 grams  $ZrO_2$ , 50 grams colloidal alumina and 2500 grams isopropyl alcohol. The coating was applied by dipping each end of sealed arc tube 1 into the dark coating suspension, removing the excess from press seal 2 and then firing the coating, for example, at 550°C to 800°C, to improve its adhesion. The second coating was applied over the first coating by also dipping the arc tube ends into the  $ZrO_2$  suspension, removing the excess from press seal 2 and firing the coating.

Although this invention is applicable to the use of any suitable heat absorbing material, such as carbon black, for the first layer of coating 9, there is particular advantage to the use of  $ZrB_2$  or a mixture of  $ZrB_2$  and  $ZrO_2$ . A suitable material has a high melting point and a low vapor pressure at the normal operating temperature of the arc tube, that is to say, it does not emit gas during normal lamp operation.

Under the conditions to which coating 9 is exposed during lamp operation, there is a gradual decomposition of the  $ZrB_2$ ; a borosilicate glass and zirconium metal are the end product. Borosilicate glass is transparent while the zirconium metal can act as an oxygen getter and form  $ZrO_2$ , which is the white reflective coating normally used on an arc tube. This reaction takes place while tungsten blackening occurs within the arc tube. With the external coating becoming lighter while a dark inner coating forms, the temperature characteristics affecting condensate are far more stable

than in prior art lamps. This results in a discharge which shows very little color change throughout lamp life. This is significant since the human eye is far more sensitive to color variation than it is to absolute intensity. Spectroscopic data have confirmed that lamps made in accordance with this invention and operated for 6000 hours show spectral radiation very similar to a new lamp, with little change in either arc temperature or color temperature. Prior art lamps operated for 6000 hours exhibited the characteristic shift toward a pure mercury lamp, with the associated increases in both arc temperature and color temperature. This indicates that lumen losses in the lamps of this invention are almost entirely due to interior arc tube wall blackening, while such blackening, together with condensate losses, affect both the output and the color of the radiation from prior art lamps.

The emittance of various mixtures of  $ZrB_2$  and  $ZrO_2$  was measured in the infrared to determine their relative efficiency as heat absorbers. The usual white  $ZrO_2$  coating of the prior art has an emittance of 0.36 (reflectivity of 0.64) while a coating of  $ZrB_2$  has an emittance of 0.96. Mixtures of  $ZrB_2$ - $ZrO_2$  containing 12½%, 25%, 50% and 75%  $ZrB_2$  have emittances, respectively, of 0.72, 0.91, 0.95 and 0.96. Thus a mixture containing 25%  $ZrB_2$  is almost as efficient a heat absorber as  $ZrB_2$  alone.

We claim:

1. An arc discharge lamp comprising an arc tube, made of high silica glass and having press seals at each end, containing a filling including inert starting gas, mercury and metal halide, having electrodes sealed therein at opposite ends and having a coating on the ends of said arc tube, said coating comprising a first layer of a dark or gray heat absorbing material and a second layer of a white heat reflecting material, said dark or gray heat absorbing material comprising zirconium diboride.

2. The lamp of claim 1 wherein the first layer comprises a mixture of zirconium diboride and zirconium dioxide.

3. The lamp of claim 3 wherein zirconium diboride comprises at least 12½% of said mixture.

4. The lamp of claim 3 wherein zirconium diboride comprises at least 25% of said mixture.

5. The lamp of claim 1 wherein said second layer comprises zirconium dioxide.

6. The lamp of claim 1 wherein said first layer comprises a mixture of  $ZrB_2$  and  $ZrO_2$  and said second layer comprises  $ZrO_2$ .

\* \* \* \* \*